

## UNITED STATES PATENT OFFICE

2,635,059

RESIN-IMPREGNATED WATER-RESISTANT  
LEATHERNicholas D. Cheronis, Chicago, Ill., assignor of  
one-third to Edwin L. Gustus, Chicago, Ill.No Drawing. Application October 26, 1948,  
Serial No. 56,663

8 Claims. (Cl. 117—135.5)

1

This is a continuation-in-part application of my copending application Serial No. 613,009, filed August 27, 1945 (now abandoned).

My invention relates to a new and novel leather and to its preparation. More particularly, it relates to a method of making fibrous materials, and especially leather, water-resistant without harmfully affecting its other characteristics, and to the leather or other fibrous material thus produced. My method is particularly advantageous for leather, but may be used upon fabrics, webbing, and other fibrous products.

A specific object of my invention is to produce leather which is water-resistant, yet flexible, soft, tough, long-wearing and more resistant to heat and cold than are conventional treated leathers.

Another object of my invention is the treatment of leather and other fibrous materials with novel aminosilane resins described and claimed in my copending (at the time of filing my present application) applications Serial No. 616,475, filed September 14, 1945, and Serial No. 72,548, filed January 24, 1949. Application Serial No. 616,475 has been abandoned in favor of application Serial No. 72,548.

Application Serial No. 72,548 has now matured into Patent No. 2,579,418, granted December 18, 1951.

A further object of my invention is to prepare solutions and dubbing which will impart water-resistant characteristics to leather or other fibrous material upon which used.

A still further object of my invention is a method of treating leather so as to make it water-resistant without deleteriously affecting the other properties of the leather which make it desirable for specific uses.

In the past, conventional water-proofing treatments for leather have been largely methods for filling the porous structure of the leather so as to render it impervious. Among the first of the methods was the old farm method of filling the leather with mutton suet. Since then other greases and waxes have been used, largely with the same intent of coating the leather microscopically. At the same time, the leather so treated was rendered especially susceptible to heat and cold because the fluidity of the grease and wax was changed greatly with only a small change in temperature. Boots treated with such grease were so stiff when cold that users would be forced to warm their boots in order to put them on. The prior methods consisted largely of providing a grease or other coating which rendered the leather water-resistant only be-

2

cause the water could not penetrate the coating on the leather, and was effective only until the coating was fractured. My method on the contrary makes each fiber in itself more water-repellent so that the water must penetrate each individual fiber to affect that fiber, and as it does not form an impervious coat to exclude the water, the leather remains porous.

My method renders the leather water-resistant, without rendering the leather impermeable. The degree may be varied by the quantity of compound used so that if desired, sufficient can be added to form a vapor-impermeable leather, but such is not ordinarily desired.

My invention provides a method of treating the leather so that the fibers themselves are water-resistant to such an extent that they repel water even when flexed repeatedly, and the leather is soft and flexible to practically the same extent as the untreated leather, yet will resist the effects of water to a far greater extent. My method will not waterproof leather to the extent that a sheet of rubber is waterproof, but will increase its resistance to water so that the leather will exhibit up to ten or more times as much resistance on standard water-resistance tests as will the untreated leather, and still remain water-vapor permeable.

The treatment is particularly useful for gloves and other leather articles in which water-resistance is at a premium, but in which the natural flexibility and toughness of the leather must be retained. Any leather may be treated, and its water-resistance increased. The final properties of the leather will be largely those of the untreated leather except for the water-resistance, and accordingly, by a suitable initial choice of leather the treated leather may be used for any purpose for which leathers are desired.

Further, a dubbing prepared in accordance with my invention may be used for maintenance of my leather, and for the increasing of water-resistance and flexibility of conventional leather.

By my invention, leather of any desired quality is treated with a solution or dispersion of certain aminosilane resins containing suitable modifiers, plasticizers and extenders, wherein the leather is impregnated with the resin at an intermediate stage of polymerization in which the resin is of low molecular weight and soluble in organic solvents. The solvent is removed by evaporation, and the polymerization of the resin is completed. The process possesses important differences from known processes, because of polymerization is completed in the final location rather than prior to treatment, and because of

the fact that the polymer is not a coating but is formed as uniformly as practicable throughout the leather structure and subsequent to tanning. The aminosilane resins polymerize by deaminative condensation, that is by elimination of a molecule of ammonia from two reactive amino groups of low molecular weight aminosilanes:



10

The monomer is not believed to be capable of existence in the free state. When  $n$  is 1, i. e., when  $n$  is one monovalent radical substituent on the silicon atom of the starting material, the resulting condensation product will thus be



R

i. e., the atomic ratio between silicon and nitrogen will be 1:1.5, the fractional number of nitrogen atoms being due to the sharing of the  $NH_2$  group by adjacent cross-linked organosilicon groups.

Deamination occurs at comparatively moderate temperatures; consequently the completion of the polymerization in situ is non-injurious to the leather. Solutions and dispersions of the aminosilane resins and their mixtures with other resins in the incompletely polymerized state penetrate into the leather so as to give the desired qualities when polymerized. As a specific example, a suitable impregnant was prepared by heating, by weight, 15 parts of coumarone indene resin, having a melting point of about 105-110° C., 20 parts of oil of oiticica, and 8 parts of linseed oil to a temperature of 200° C. for 15 minutes, then adding 20 parts of paraffin wax. Separately, a mixture was prepared of 10 parts tricresylphosphate, 6 parts light paraffin oil, and 4 parts blown castor oil. Separately, 20 parts of styrene was heated to 135° C., 0.2 part of benzoyl peroxide was added in small portions so as to keep the styrene near boiling as it polymerized. The polymerization was allowed to continue until the viscosity increased to between 30 and 34 poises at 20° C. A solution was prepared of ethyl aminosilane resins by allowing a solution of 117 grams of ethyl trichlorosilane (technical) in 200 grams of dry xylene to react with 200 ml. of liquid ammonia, filtering out the ammonium chloride, washing with 200 ml. of dry xylene and evaporating off the surplus ammonia under vacuum. As prepared, the solution contained about 16% of the resin intermediate. A quantity of this solution containing 20 parts solids was mixed with the other three solutions. The resulting solution was diluted by the addition of xylene and mineral spirits so that the final concentration of solids was between 20-30%.

The solids content of the solution may vary from 5% to 30% depending on the "add-on" that is desired; for most purposes a content of 18 to 20% is used. Where it is intended to emulsify the resin solution prior to its application to leather, the solids concentration is preferably from 20 to 25% based on the weight of the emulsion; this is diluted in the mill to a preferred solids concentration of from 7 to 14%. The ratio of organoaminosilane resins to the rest of the solids may vary between 10 to 90%, but it is particularly desirable that it range from 10 to 40% of the total solids; thus the organoaminosilane resin content of the solution may vary from 5% to 27%, and preferably from 5 to 12%. 75

If it is desired to store the solution for a period before use, an inhibitor may be used to slow down the rate of polymerization of the silicon-free polymerizable components of the solution. Volatile inhibitors, such as cyclohexylamine, benzylamine, n-butyl amine, tributyl amine, dicyclohexylamine, or aryl amines such as benzylamine, etc., may be used. An amount of from 0.5% to 2% of the weight of the resins is usually satisfactory. When a non-volatile accelerator is present in one of the component monomers, it may be left in the solution as the dilution in xylene usually arrests polymerization to an adequate degree.

A deerskin glove leather was treated by dipping in the solution for 30-40 seconds, drying to evaporate the solvent and curing at 60-65° C. for 24 hours (or for 4 hours at 60-65° C. followed by 24 hours at room temperature), during which time condensation and polymerization was completed. The weight of deposited solids ranges from 20-30% of the original weight of the leather.

During the impregnation with the resin, a portion of the oil or fat which the leather contains was extracted by the highly aromatic solvent used for the resins, and oil or fat should be replaced to keep the leather soft. Ordinary shoe dubbing is satisfactory, but a better one is prepared by including such highly water-repellent components as 5% octadecylamine and about 5% silicon amine resin which has been previously polymerized. For example, the dubbing may consist of:

|                       | Parts |
|-----------------------|-------|
| Beef tallow           | 20-40 |
| Animal oil            | 20-30 |
| Amorphous mineral wax | 8-10  |
| Silicon amine resin   | 10-30 |
| Octadecylamine        | 5-10  |
| Aluminum stearate     | 1-2   |

The solution to be used in the treatment of the leather comprises an aminosilane compound obtained from the ammonolysis of organosilicon halides, either pure or mixed, where the degree of halogenation is sufficiently high to give polymerizable compounds; at least two valences of the silicon must be substituted by halogen atoms in order that polymerized aminosilanes may be obtained. Such compounds are methyl trichlorosilane, dimethyl dichlorosilane, ethyl trichlorosilane, diethyl dichlorosilane, methyl ethyl dichlorosilane, phenyl trichlorosilane, diphenyl dichlorosilane, phenyl methyl dichlorosilane, ethyl trifluorosilane, ethyl triiodosilane, etc. The term "ammonolysis" includes reactions with not only ammonia, but also with substituted ammonia, such as the primary amines, methyl amine, butyl amine, isobutyl amine, phenylamine, hexamethylene diamine, ethylene di- and polyamines, etc. It is possible that during the final polymerization step in situ nitrogen of the amino groups of the resinous product form secondary linkages with the protein fibers and thus serve as anchorages for the resin. The resulting resinous products are characterized by a silicon to nitrogen ratio of from 1:1 (approximately) to 1:1.5 (approximately); they are further characterized by repeating units of silicon linked to nitrogen as an integral part of the polymer chain in which the repeating units consist of silicon substituted by monovalent hydrocarbon radicals, as is more fully explained in my copending application 616,475. Other components of the solution comprise one or more of the following: (a)

résins already "preformed" (completely polymerized), as coumar resin, ester gum, rosin, rosin modified phenolic, maleic-resin, (b) unsaturated glycerides of the type of China-wood oil, oil of oiticica, perilla, linseed etc., partially polymerized by heating to a certain viscosity, (c) plasticizers such as dibutyl phthalate, tricresyl phosphate, etc., (d) a partially polymerized resin-forming material, such as styrene, coumar, coumarone indene, modified Bakelite, etc.

A particularly preferred solvent consists of a mixture of xylene and mineral spirits in the ratio of about 4:1. Other suitable solvents are xylene, toluene, benzene (to be used with caution because of the toxicity of its vapors), high boiling point ethers such as butyl ether, Stoddard solvent; amyl or butyl alcohol in suitable amounts say 10%, may be added to the inert solvents. Other suitable solvents which are non-settling, economical, and non-reactive with the aminosilane resin will readily occur to the expert in the art in the light of the foregoing disclosure.

The organoaminosilane resins may be used either alone, or in conjunction with other resinous water-repellent materials to treat leather. If they are used alone, the type of aminosilane resin must be selected so that when it is cured it will yield a soft flexible non-tacky resin. This can be accomplished by increasing the ratio of di-functional monomer and decreasing the ratio of the tri-functional monomer in the mixture which is to be ammonolyzed. For example, if the mixture ammonolyzed consists of 95% trihalosilane ( $RSiCl_3$ ) and 5% dihalosilane



the resulting resin will have a considerable number of cross links between relatively short chains and hence will have a tendency to brittleness and granulation under dynamic conditions. On the other hand, if the mixture ammonolyzed consists of 80% or 70% or 60% or 50% tri-functional, and 20% or 30% or 40% or 50% di-functional the resulting resins will have a tendency toward softness and flexibility. On the other hand, as the amount of the di-functional monomer is increased the ease at which the resins "cure" at room temperature by evolution of ammonia decreases. In other words, it will require heat to effect curing. However, it is clear that by controlling the ratio of the tri-functional and di-functional halosilanes of the ammonolyzed mixture, it is possible to obtain a series of resins which after curing will vary all the way from the oily type to the hard brittle type. The particular type of resin to be used depends on the ultimate use. If the leather to be treated is sole leather, a hard, tough and slightly resilient resin must be used since the flexing is at a minimum. On the other hand for glove leather, a soft non-tacky resilient resin is required.

It has been found out by actual experimentation that the amount of aminosilane resin to be introduced into leather need not be very high. For example, in order to obtain leather of high degree of water repellency, it is necessary first to coat the fibers and fiber-bundles which make up the leather so as to stop their "wicking" action; at the same time, however, the interfiber spaces must be filled so as to reduce the empty or void spaces and therefore reduce the amount of water which will tend to be forced by pressure under flexing into the leather pores or empty spaces. The silicon resins are ideal for coating the fibers and fiber-bundles so as to impart a high

degree of water repellency. Although it is possible to coat the fibers in the interior of the leather with silicon resins alone, the cost of such a process is likely to be rather high because of the present price of silicon resins; therefore it is advantageous to add other polymeric substances to the silicon polymer containing leather treating composition. Therefore if the silicon resin makes up between 10% and 40% of the total film which has been deposited within the leather, the performance of the leather is as good and in some cases superior to leather treated with silicon resins alone.

The selection of the materials to be introduced into leather in conjunction with the aminosilane resins should have the following characteristics: (a) they should not react with the aminosilane resins before the curing period; (b) they should be compatible with the aminosilane resins after curing; in other words they should not separate as a separate film after curing, but should form either a solid solution or a compound with the silicon resin; (c) they should have a comparatively low molecular weight prior to curing so that they can be introduced in the same way as the aminosilane resins, and they should be capable of further polymerization after deposition in the same manner as the aminosilane resins.

Certain polymeric substances fulfill these requirements. They are made from monomers and are "incompletely polymerized," that is, they are polymerized until they form liquid low molecular weight polymers capable of still further polymerization; the polymerization is then arrested, e. g. by the use of a suitable inhibitor, examples of which are set forth above. Under these conditions of preparation, these "partial polymers" have the following characteristics: (a) they are liquid at room temperatures of viscosity of 3-60 poises; (b) are soluble in a variety of organic solvents; (c) are stable and can be stored for long periods of time; (d) are capable after deposition and evaporation of the solvent and inhibitor to polymerize further and thus form an "anchored" film, that is, a film firmly bonded to the impregnated base.

For the preparation of the "partial polymer" which can be used in conjunction with the aminosilane resins, the following monomers have been used either alone or in mixtures: methyl acrylate, ethyl acrylate, butyl acrylate, octyl acrylate and lauryl acrylate; methyl methacrylate, butyl methacrylate, lauryl methacrylate; styrene; chlorostyrene, vinyl acetate, vinylidene chloride.

Another type of polymerizable film that can be used in conjunction with the aminosilane resins is a film produced by polymerization of a mixture of oxidizable unsaturated glycerides or drying oils and resins. For example a mixture of oils of oiticica, China-wood, and linseed oil heated with a coumarone indene resin or phenol-formaldehyde resin is an example of this type of polymerizable film. Equal parts of oils and resins are heated to about 200° C. until the required degree of polymerization of the unsaturated glycerides has taken place and then are allowed to cool to room temperature when they can be mixed with the aminosilane resin, or mixture of aminosilane resin and "partial polymeric" material.

No matter what the composition of the resin is, it should be plasticized in order that the required degree of the flexibility is obtained. The nature of the plasticizer must be such that it is compatible and non-reactive with the amino-

silane resin and also compatible with the other type of materials which are introduced in conjunction with the aminosilane resins. Among those useful for this purpose are: esters of phosphoric acid, such as cresyl phosphates, butyl phosphates; esters of phthalic acid, such as butyl phthalate, octyl phthalates and the like; esters of glycerol and glycol; oils such as castor oil and neat's-foot oil; low melting point paraffin wax (M. P. 60-65° C.). The amount of plasticizer to be used depends on the type of leather treated. Generally the amount of plasticizing is minimum in sole leather treatment and maximum in glove leather treatment.

Once the nature of the composition of the mixture to be introduced into leather has been made, a choice must be made as to the method of introduction. Generally there are two methods (a) non-aqueous solution method; (b) aqueous emulsion method. In the non-aqueous solution method, the aminosilane together with any other film producing substances or mixture of substances such as "partial polymers," resin-oxidizable oil mixture and the like, are dissolved into an organic solvent such as xylene, toluene, or mixtures of xylene, aliphatic naphtha, and alcohols. The strength of the solution is adjusted depending on the deposition required. For example, if a 25-30% deposition of solids by weight of leather is required the solution should contain 40% of solids. On the other hand if only a 10% deposition is required, a 15% solution is adequate. The leather may be treated by dipping, sponging, or spraying. In any case the excess of the solution is drained or removed by centrifuging and the skin is placed in a dryer for removal of the solvent and curing. The temperature required is 110 to 140° F. or 55-65° C. During the first hours of the heating the solvent and inhibitors evaporate and the polymerization in situ begins. The time required for complete curing varies with the nature of the aminosilane resin used, the nature of the "partial polymers." If no oxidizable oil-resin mixture has been used, the curing is substantially complete within 4 hours; if the amount of di-functional monomers in the aminosilane resin is high, the curing will take longer; if oxidizable oil-resin mixture has been used, the skin is allowed to stand at room temperature for 48 hours after the initial heating when the oxidizable phase is complete. The curing in the case of the aminosilane resins which have high ratio of tri-functional monomers can be completed speedily within a few minutes at 90° C. or slowly at room temperature for two days. However, it has been found that an initial heating period of a few hours at about 60° C. followed by standing at room temperature for overnight is better than curing at temperatures of above 70° C. for lesser periods of time, since above the latter temperature, there is danger for the leather to be harmed if supervision of the curing is not carried out with meticulous care.

In the aqueous emulsion method, the aminosilane resin or aminosilane resin mixed with partial polymeric resins are dissolved in a water-insoluble organic solvent of the hydrocarbon type such as xylene, toluene and the like. Small amounts of alcohol, ethers, ketones, may be used but not to exceed 10-15% of the total amount of the solvent used since emulsification becomes difficult if appreciable amounts of polar solvents are present. The

amount of solvent used is preferably adjusted so that the solvent content in the final emulsion is 25-40%. The presence of the solvent is necessary for the success of this process and although it is possible to emulsify the resin-oil mixture without the presence of the solvent the resultant emulsion deposits most of the resins on the surface and outer layers of the leather, instead of penetrating the interfiber space of the leather and uniformly distributing the deposited film.

After the liquid aminosilane resins and other "partial polymers" are dissolved then they are emulsified by special types of emulsifying agents which give a dispersion or emulsion having the desired characteristics which are: (a) the emulsion should not be so unstable that it breaks suddenly when it is brought in contact with the skin, thus depositing the resinous materials on the outer surface of the leather; (b) on the other hand, the emulsion should not be so excessively stable so that it will require several hours of tumbling it with the skin in the leather mill so that it may break, for in such case the leather is damaged by too much tumbling; (c) the emulsion should break within 15-45 minutes after coming in contact with the wet skin, and in so breaking the emulsified particle should slip between the fiber-bundles within the leather and there be discharged depositing the organic particle in exchange with water. In other words, the wet skin gives up water in exchange for organic particles. The organic particles consist of droplets of solvent containing resins; as the solvent evaporates (and the evaporation starts within the mill since the temperature during the operation is about 100 to 120° F.) the deposition of the film takes place. This deposition is more uniform and more penetrating than treatment with a solvent. After the skin has been treated with the emulsion then it is placed into a room heated to 120-130° F. and allowed to stay 24 to 48 hours. During this time the water evaporates and the polymerization or curing is completed. Further details of leather treatment by contact with an emulsion containing a solution of silicon amine resin are set forth in my copending application Serial No. 643,493, filed January 25, 1946.

Each method of introduction has some advantages and some disadvantages. For example, of finished articles such as gloves, shoes, straps, which have been already manufactured, the solvent method is used. On the other hand, the emulsion method is better adaptable to large scale tannery operation, since it removes the hazard due to flammable solvents and leads to a more uniform deposition and at the same time utilizes machinery which every tannery has. It should be stated, however, that in utilizing the aqueous emulsion method the aminosilane resin must be selected from the type that hydrolyzes with water very slowly. For example, an aminosilane resin made from mixtures of dimethyltrihalosilane and methyltrihalosilane undergoes rapid hydrolysis and hence cannot be used successfully with the emulsion method; on the other hand, an aminosilane resin derived from the ammonolysis of phenyltrihalosilane and diphenyldihalosilane undergoes very little hydrolysis over the period of time required for emulsion operation, and hence it can be used with the emulsion method. Such aminosilanes that are subject to rapid hydrolysis can be used successfully by the non-aqueous solvent method.

The following examples illustrate some of the principles discussed in the preceding paragraphs:

## FORMULA A

## Aminosilane with partial polymers

|                    | Parts |
|--------------------|-------|
| Butyl acrylate     | 30    |
| Butyl methacrylate | 25    |
| Styrene            | 11    |
|                    | —     |
| Total monomer      | 66    |

Heat to 125° C. and add slowly over a period of 15 minutes 0.5 part of benzoyl peroxide and continue heating until the viscosity of the liquid intermediate polymer is 10 to 15 poises at 25° C. Now add 0.1 part of cyclohexylamine as inhibitor and dilute with xylene or toluene to 200 grams thus obtaining a stable solution. Cool to room temperature and add:

Aminosilane resin, 30 parts (from the ammonolysis of a mixture of 60 parts of ethyltrichlorosilane and 40 parts of diethylchlorosilane)  
Octyl phthalate (plasticizer), 14 parts  
Solvent sufficient to make up a solution which has 25% solids.

## FORMULA B

## Aminosilane resin with partial polymers

|                                               | Parts |
|-----------------------------------------------|-------|
| Styrene monomer                               | 10    |
| Vinyl acetate                                 | 10    |
| Methyl methacrylate                           | 10    |
| Butyl acrylate                                | 30    |
| Benzoyl peroxide                              | 0.8   |
| Polymerize to 12-15 poises viscosity and add: | 40    |
| Cyclohexylamine                               | 0.2   |
| Paraffin wax                                  | 10    |
| Tricresyl phosphate                           | 10    |
| Aminosilane resin                             | 20    |

The aminosilane resin was produced from the ammonolysis of 80 parts of phenyltrichlorosilane and 20 parts of diphenyldichlorosilane, as set forth in Example 8 of my copending application Serial No. 72,548 (which example is in turn based on Example 6 of my application Serial No. 56,662, filed October 26, 1948, and now abandoned in favor of my application No. 72,548.) For an example of a treatment by the solution method enough xylene is added to give a 25% solution. For an example of a treatment by the aqueous emulsion method the 100 parts of the mixture are dissolved into 180 parts of xylene and then 5 parts of sulfated neat's-foot oil and 5 parts of a commercial emulsifier such as a sodium salt of a higher synthetic alcohol sulfate, known by the trade name of "Tergitol," e. g. ("Tergitol Penetrant 4" which is the sodium salt of 7-ethyl-2-methyl-undecanol-4-sulfate), are added and then emulsified by mixing with 220 parts of water and passing through a colloid mill. About 500 parts of emulsion are obtained containing 20% of solids and having a pH of 9.2 to 9.5. Such emulsion should be used immediately after preparation. For use it is diluted with an equal amount of water heated to 50° C. and then added to the leather mill containing the wet skin. Exhaustion is substantially complete within 30-45 minutes. The spent liquor is substantially free of any polymer thus showing complete absorption.

## EXAMPLE C

## Aminosilane resin with partial polymers and oxidizable oils

## 5 Aminosilane resin, 20 parts

(Obtained by the ammonolysis of 70 parts of phenyltrichlorosilane and 30 parts dimethyl-dichlorosilane)

10 10 Partial polymeric resin mixture, 35 parts  
Composition: butyl methacrylate 15 parts, styrene 10 parts, vinyl acetate 10 parts, benzoyl peroxide 0.15 part; polymerized to 10-12 poises viscosity and inhibited with 0.05 part cyclohexylamine.

## 15 Oxidizable oil-resin mixture, 35 parts

Composition: Indene-coumarone resin 15 parts; oil of oiticica 14 parts, linseed oil 3 parts, heated to 200° C. for 20 minutes and then cooled to 100° C. and mixed with 3 parts of paraffin wax and 0.1 part of 6% cobalt naphthenate (drier)

## 20 Plasticizing mixture, 10 parts

Composition: castor oil 3 parts, tricresyl phosphate 3 parts, and octyl phthalate 4 parts.

25 Sufficient solvent is added (xylene or toluene) to give a solution having 15-30% of solids.

Proof that the aminosilane resin is actually deposited as such in the leather as such as not 30 hydrolyzed is shown by the following examples:

## EXAMPLE 1

35 A piece of upper leather weighing 810 grams gave on analysis 8.61% of nitrogen which corresponds to 54.61% of hide substance. The grease content was 22%. This piece of leather was treated with solution of Formula A and after curing it was found to weigh 1014 grams, a gain of 25.2%. On that basis of gain if there had been no nitrogen introduced the percentage of nitrogen in the leather would be about 6.9%. However, on analysis the leather gave 7.65%, a gain of 0.75%. In addition, the leather contains silicon as shown by analysis for silica in 45 the ash. The amount of silica found was 1.7%.

## EXAMPLE 2

Treatment of a hide by the emulsion method. A horsehide was used weighing 960 grams containing 11% of grease. The hide was first chrome-tanned and then fat-liquored so that 50 11% of oil was absorbed. The leather was then used directly for the emulsion treatment in order to introduce the aminosilane resin. This organosilicon resin was made by ammonolysis of a mixture made of 0.6 mol. of phenyltrichlorosilane and 0.4 mol of diphenyldichlorosilane. The aminosilane resin was introduced into a formula of Type B and then converted into an aqueous emulsion as described. Exactly 1500 grams of the emulsion containing 20% solids were added to the mill together with 1500 grams of water. Both the water and the emulsion were heated to 60° C. before addition. The wet skin was added 55 and tumbled for 50 minutes. The pH of the spent liquor was 6.2. The skin was removed and placed in the hot room (110-120° F.) for 48 hours and then staked as usual. The dry skin weighed 1245 grams, a gain of 29.5%. The analysis for nitrogen before and after showed an increase in the nitrogen content by 0.54%.

The degree of water-resistance of the leather depends upon the type and amount of resins used. Normally the water vapor permeability of the 60 65 leather should not be drastically reduced. The 75

upper limit of solids from resin dispersion, including the plasticizer, modifier, softeners, etc., is around 30-40 by weight based upon the untreated weight of the leather. However, where permeability is not important, as in leather straps, belts, etc., the leather can be impregnated to 50% solids or more advantageously. In gloves, from 15-30% by weight is a desirable range. However, the value of the resin treatment varies with the amount of solids, and is quite marked even when as low as 5% is deposited. A higher percentage of aminosilane resin, particularly of the di-functional type, increases the flexibility and the stretch of the leather, especially in cold climates. The aminosilane resins permit the use of a lower ratio of plasticizer, etc., give particularly desirable products. For some leather ease of curing conditions is critical, and for all leathers, it is desirable, as undue heating can become harmful to the leather. The deamination polymerization of aminosilane resins takes place at lower temperatures than the dehydrogenation polymerization of silicone resins, due to the low boiling point of ammonia; this property is therefore particularly desirable in the application of aminosilane resins to leather.

Thus the amount of solids deposited in the leather from a resin solution, ranges from about 5% to 50% based on the total weight after treatment; for most practical purposes I prefer 10%-30%. The amount of organosilicon amine resin "add on" in the leather accordingly ranges from 5% to 45%.

The amount of solids deposited in the leather by emulsion treatment ranges from about 10% to 45% based on the weight of the impregnated leather; a highly desirable leather is obtained with a solids deposition of about 30 to 40% from an emulsion.

The Si content of leather treated with the organosilicon amine resin solution or emulsion may be as little as .2% of the Si content, untreated leather being .04%. By saturating the leather with a concentration of 45% silicon amine resin intermediate, I have succeeded in raising the Si content of heavy duty leather to 11.5%. However, for most practical purposes, I have found a Si analysis of 1.4% to 2.3% to be sufficient to impart the desired water-resistance and suppleness to the leather.

The degree of "partial polymerization" before impregnation can be determined by viscosity tests or by cryoscopic average molecular weight determination; the organosilicon amine resin intermediates, in their partially polymerized state prior to application of the resin to the leather, are organic-solvent-soluble liquids at ordinary temperatures, which unless stabilized will in time polymerize to form solid resins. Their viscosity is from 3 to 60 poises at 20° C. Generally these partially polymerized intermediates have from 3 to 60 repeating units; I prefer to utilize those intermediates whose viscosity at 20° C. lies between 3 and 12 poises, and especially those between 4 and 8 poises. Molecular weights of the organosilicon amine resin intermediates may be up to 5000, depending on the molecular weight of the monomer; their average molecular weight usually varies from 250 to 1600, and, in my preferred range, it is between 400 and 800.

I claim:

1. In a method of imparting water-resistance to an air-permeable fibrous material, the steps which comprise: impregnating said fibrous material with a solution, in an inert volatile organic

solvent, of an incompletely polymerized liquid silicon amine resin characterized by repeating units of silicon linked to nitrogen as an integral part of the polymer chain in which the repeating units consist of silicon substituted by from one to two monovalent hydrocarbon radicals, said silicon being attached to nitrogen substituted by a member of the group consisting of hydrogen and hydrocarbon radicals, at least half of said repeating units being substituted by only one of said monovalent hydrocarbon radicals per silicon atom, said silicon amine resin being polymerized to a liquid capable of further polymerization to a solid and having in the free state a viscosity of from about 3 to about 60 poises measured at 20° C., the amount of dissolved silicon amine resin deposited in said fibrous material being between about .5% and about 45% of the weight of said fibrous material; and further polymerizing said resin in the interfiber space of said fibrous material at a temperature not exceeding about 90° C. to form a solid coating of said silicon amine resin on the individual fibers of said fibrous material so as to make said fibrous material water-resistant without destroying its air-permeability.

2. In a method of imparting water-resistance to an air-permeable fibrous material, the steps which comprise: impregnating said fibrous material with a solution, in an inert volatile organic solvent, of an incompletely polymerized liquid silicon amine resin characterized by repeating units of silicon linked to nitrogen as an integral part of the polymer chain in which the repeating units consists of silicon substituted by one monovalent hydrocarbon radical, said silicon being attached to nitrogen substituted by a member of the group consisting of hydrogen and hydrocarbon radicals, said silicon amine resin being polymerized to a liquid capable of further polymerization to a solid and having in the free state a viscosity of from about 3 to about 60 poises measured at 20° C., the amount of dissolved silicon amine resin deposited in said fibrous material being between about .5% and about 45% of the weight of said fibrous material; and further polymerizing said resin in the interfiber space of said fibrous material at a temperature not exceeding about 90° C. to form a solid coating of said silicon amine resin on the individual fibers of said fibrous material so as to make said fibrous material water-resistant without destroying its air-permeability, said further polymerized silicon amine resin having an average ratio of 1 atom of silicon to approximately 1.5 atoms of nitrogen in its repeating units.

3. In a method of imparting water-resistance to leather, the steps which comprise: impregnating said leather with an aqueous emulsion of a solution, in an inert volatile organic solvent, of an incompletely polymerized liquid silicon amine resin characterized by repeating units of silicon linked to nitrogen as an integral part of the polymer chain in which the repeating units consist of silicon substituted by from one to two monovalent hydrocarbon radicals, said silicon being attached to nitrogen substituted by a member of the group consisting of hydrogen and hydrocarbon radicals, at least half of said repeating units being substituted by only one of said monovalent hydrocarbon radicals per silicon atom, said silicon amine resin being polymerized to a liquid capable of further polymerization to a solid and having in the free state a viscosity of from about 3 to about 60 poises measured at 20° C., the amount of

dissolved silicon amine resin deposited in said leather being between about .5% and about 45% of the weight of said leather; breaking said emulsion inside said leather; and further polymerizing said resin in the interfiber space of said fibrous material at a temperature not exceeding about 90° C. to form a solid coating of said silicon amine resin on the individual fibers of said leather so as to make said leather water-resistant without destroying its air-permeability.

4. The method according to claim 3, wherein said emulsion is broken inside the leather by tumbling said leather.

5. A water-resistant air-permeable fibrous material whose individual fibers carry a solid coating of a silicon amine polymeric resin characterized by repeating units of silicon linked to nitrogen as an integral part of the polymer chain in which the repeating units consist of silicon substituted by from one to two monovalent hydrocarbon radicals, said silicon being attached to nitrogen substituted by a member of the group consisting of hydrogen and hydrocarbon radicals, at least half of said repeating units having only one said monovalent hydrocarbon radical substituent per silicon atom, said coating being formed on said individual fibers by the method of claim 1.

6. A composition for imparting water-resistance to fibrous materials comprising a solution in a common inert volatile organic solvent, of an incompletely polymerized liquid silicon amine resin characterized by repeating units of silicon linked to nitrogen as an integral part of the polymer chain in which the repeating units consist of silicon substituted by from one to two monovalent hydrocarbon radicals, said silicon being attached to nitrogen substituted by a member of the group consisting of hydrogen and hydrocarbon radicals, at least half of said repeating units being substituted by only one of said monovalent hydrocarbon radicals per silicon atom, said silicon amine resin being polymerized to a liquid capable of further polymerization to a solid and having in the free state a viscosity of from about 3 to about 60 poises measured at 20° C., and of an incompletely polymerized organic-solvent-soluble liquid polymer of a member of the group consisting of alkyl acrylate, alkyl methacrylate, styrene, chlorostyrene, vinyl acetate, and vinylidene chloride, and capable of further polymerization to a solid; the proportion

of said silicon amine resin being between 10% and 90% of the total amount of polymers in said composition.

7. A leather treating composition according to claim 6, wherein the proportion of said silicon resin is between 10% and 40% of the total amount of polymers in said composition.
8. A leather-treating composition comprising in a common inert volatile organic solvent: an incompletely polymerized liquid copolymer of styrene and of a member of the group consisting of alkyl acrylate and alkyl methacrylate, and an incompletely polymerized silicon amine resin characterized by repeating units of silicon linked to nitrogen as an integral part of the polymer chain in which the repeating units consist of silicon substituted by from one to two monovalent hydrocarbon radicals, said silicon being attached to nitrogen substituted by a member of the group consisting of hydrogen and hydrocarbon radicals, at least half of said repeating units being substituted by only one of said monovalent hydrocarbon radicals per silicon atom, said silicon amine resin being polymerized to a liquid capable of further polymerization to a solid and having in the free state a viscosity of from about 3 to about 60 poises measured at 20° C.; the proportion of said silicon amine resin being between 10% and 90% of the total amount of polymers in said composition.

NICHOLAS D. CHERONIS.

References Cited in the file of this patent

UNITED STATES PATENTS

| Number       | Name         | Date          |
|--------------|--------------|---------------|
| 1,952,137    | Muller       | Mar. 27, 1934 |
| 2,258,220    | Rochow       | Oct. 7, 1941  |
| 2,280,830    | Johnson      | Apr. 28, 1942 |
| 40 2,306,222 | Patnode      | Dec. 22, 1942 |
| 2,356,879    | Pense et al. | Aug. 29, 1944 |
| 2,364,692    | Cassel       | Dec. 12, 1944 |
| 2,377,689    | Hyde         | June 5, 1945  |
| 2,385,800    | Douty et al. | Oct. 2, 1945  |
| 45 2,392,805 | Biefeld      | Jan. 15, 1946 |
| 2,462,635    | Haber        | Feb. 22, 1949 |
| 2,553,314    | Haber        | May 15, 1951  |

FOREIGN PATENTS

| Number     | Country | Date          |
|------------|---------|---------------|
| 50 915,190 | France  | July 16, 1946 |